

# United States Patent Office

2,744,872

Patented May 8, 1956

1

2,744,872

## GEAR LUBRICANT COMPRISING A WIDE MINERAL OIL BLEND AND AN OXIDIZED PARAFFINIC RESIDUUM

Roy F. Nelson, Port Arthur, Tex., assignor to The Texas Company, New York, N. Y., a corporation of Delaware

No Drawing. Application June 23, 1953,  
Serial No. 363,675

6 Claims. (Cl. 252—49.6)

This invention relates to improved lubricating compositions of the fluid type, suitable for the lubrication of gears and heavy bearings. More particularly, it relates to a blend of residual and distillate mineral lubricating oils containing an oxidized paraffinic residuum.

The lubricants of this invention consist essentially of a mineral oil component comprising a wide mineral oil blend and a minor but substantial proportion, based on the composition, of an oxidized paraffinic residuum, preferably an oxidized cylinder stock residuum. The mineral oil blend comprises a substantial proportion of a heavy residual oil having a viscosity above the motor lubricating oil range and a substantial proportion of a light naphthenic oil having a viscosity in about the spindle oil range. In addition, it may comprise minor amounts of different lubricating oils of intermediate viscosities, which may be either naphthenic or paraffinic in character. The lubricant preferably comprises about 20–60 per cent by weight of heavy residual oil, having a viscosity above about 600 seconds Saybolt Universal at 210° F., about 20–60 per cent by weight of light lubricating oil having a viscosity below about 200 seconds Saybolt Universal at 100° F. and comprising in major proportion a naphthenic distillate oil having a viscosity of about 50–100 seconds Saybolt Universal at 100° F., and about 5–30 per cent by weight of oxidized paraffinic residuum having a penetration of about 30–100 and generally about 40–90 at 77° F.

Lubricants obtained by employing the above combination of materials have been found to have excellent adhesiveness to metal and other lubricating properties required of a very superior gear lubricant, suitable for use over a wide range of atmospheric temperatures and in the presence of water. They are characterized particularly by a combination of high viscosity index and low pour point, not obtainable with straight mineral oils and mineral oil blends which have been employed heretofore as transmission lubricants. Transmission lubricants are obtained in accordance with this invention having relatively high viscosities at ordinary and elevated atmospheric temperatures, such as are required to prevent gear noises, combined with very satisfactory cold starting characteristics at winter temperatures.

The residual fractions employed in these compositions are highly viscous oils, preferably of low wax content, obtained either from low wax content crudes such as naphthenic base crudes or by substantially dewaxing residual fractions from paraffinic oils. A very satisfactory residuum for this purpose is obtained from Manvel crude, which is a mixed base oil containing only about 2–3 per cent of wax and giving a residuum having a viscosity in excess of about 600 seconds Saybolt Universal at 210° F. A residuum having a viscosity of about 700–800 seconds Saybolt Universal at 210° F. is preferably employed.

The light naphthenic distillate oils employed in the compositions may be obtained by straight distillation of naphthenic type or predominantly naphthenic type crudes or by any of the usual refining methods.

The oxidized residuum is obtained by blowing a par-

2

affinic residual oil or cylinder stock residuum having a viscosity in the upper lubricating oil range, of about 90–750 seconds Saybolt Universal at 210° F., preferably having a viscosity of about 100–300 seconds Saybolt Universal at 210° F. The blowing may be carried out in the conventional manner, by blowing with air at a suitably elevated temperature of about 400–500° F. either in the presence or absence of a catalyst until a product of the desired penetration is obtained, preferably about 55–75 at 77° F. For ease in handling and compounding, the blown residuum is preferably cut back with a light mineral oil. For example, it may be suitably cut back with about 40–60 per cent by weight of a light naphthenic distillate lubricating oil having a viscosity of about 75–125 seconds Saybolt Universal at 100° F. to give a fluid oxidized residuum cut-back having a viscosity of 175–225 Saybolt Furol at 210° F. The cut back thus forms a portion of the light lubricating distillate of the final composition. The oxidized cylinder stock residuum is to be distinguished from blown asphalts prepared from asphalt-base residua heretofore employed in gear lubricants, since the oxidized cylinder stock residuum has a much higher dropping point and better temperature susceptibility than a blown asphalt because of its high paraffinic content.

As an example of the lubricating compositions of this invention, lubricants were prepared by blending together a heavy Manvel residuum with a lightly refined light naphthenic distillate oil and with a cut-back oxidized residuum, the latter consisting of a 55–75 penetration product obtained by blowing a paraffinic cylinder stock residuum having a viscosity of 120 seconds Saybolt Universal at 210° F., cut back with an equal amount by weight of a second, lightly refined naphthenic distillate oil having an SUS viscosity at 100° F. of 85–115. The oxidized residuum employed in the specific formulation No. 4 of the following Table I had a penetration of 67 and the petroleum fractions employed had the following tests:

|                             | Distillate No. 1 | Distillate No. 2 (Employed in cut-back oxidized residuum) | Residuum     |
|-----------------------------|------------------|-----------------------------------------------------------|--------------|
| Gravity, A. P. I.           | 26.5             | 23.3                                                      | 61.5         |
| Flash, C. O. C.             | 330              | 315                                                       | 700          |
| Fire, C. O. C.              | 370              |                                                           |              |
| Viscosity at 70° F., SUS    | 104.9            |                                                           | 85,000       |
| Viscosity at 100° F., SUS   | 61.3             | 123                                                       | (Calc.)      |
| Viscosity at 122° F., Furol |                  |                                                           | 1,575        |
| Viscosity at 210° F., SUS   |                  | 40                                                        | 730          |
| Viscosity index             | 16               | 48.4                                                      | 41.2         |
| Pour, A. S. T. M.           | —45              | —30                                                       | (Approx.) 60 |

The preparation of these lubricants was carried out by heating the cut back oxidized residuum employed in the compositions in a steam heated kettle to a temperature of about 150° F. and then adding the heavy residuum and the distillate oil No. 1 with continuous stirring at temperatures of about 150–175° F. In some of the preparations, a small amount of Paratac was added to the blend while the temperature was about 145° F. This is a high molecular weight linear isobutylene polymer which is employed in lubricating oil compositions to impart stringiness.

The following table shows the properties of a representative lubricant of this series (Lubricant No. 4), as compared with those of straight mineral oil blends of equivalent viscosity and penetration. Lubricant No. 1 of the table was a blend of Manvel residuum and distillate No. 2, having the properties described above. Lubricant No. 2 was a blend of a residuum having a Saybolt Universal viscosity of about 200 at 210° F., from a South Louisiana crude, which is a mixed base paraffin crude of low wax

content, with distillate No. 2. Lubricant No. 3 was a blend of the Manvel residuum with a naphthenic distillate oil having a Saybolt Universal viscosity at 100° F. of about 104, a viscosity index of about 40 and a pour point of about 10° F. Lubricant No. 5 was a commercial transmission lubricant of the blended oil type.

5 with the agitator engaged. The power consumption is measured periodically under this set of conditions. Then the test is repeated in the same manner with a 160 watt adjustment at room temperature. The ability of the unit to start and the power consumption are indicative of the suitability of the lubricant for this purpose.

TABLE II  
GE cold starting test results

| Lubricant No.                      | 1   | 2   | 3   | 4   | 5     |
|------------------------------------|-----|-----|-----|-----|-------|
| Test Conditions:                   |     |     |     |     |       |
| Watt adjustment                    | 160 | 145 | 160 | 145 | 160   |
| Room temperature, ° F.             | 75  | 75  | 80  | 81  | 83    |
| Transmission temperature, ° F.     | 31  | 33  | 33  | 32  | 33    |
| Test Results:                      |     |     |     |     |       |
| Time on starting windings, seconds | 30+ | 30+ | 30+ | 30+ | 30+   |
| Power consumption, watts, after—   | (1) | (1) | (1) | (1) | (1)   |
| 30 seconds                         |     |     |     |     | 230   |
| 1 minute                           |     |     |     |     | 200   |
| 2 minutes                          |     |     |     |     | 177   |
| 3 minutes                          |     |     |     |     | 165   |
| 4 minutes                          |     |     |     |     | 157   |
| 5 minutes                          |     |     |     |     | 150   |
|                                    |     |     |     |     | 152   |
|                                    |     |     |     |     | 1,508 |
|                                    |     |     |     |     | 1,520 |
|                                    |     |     |     |     | 35+   |

<sup>1</sup> Stalled.

<sup>2</sup> Test discontinued as drive motor was smoking.

TABLE I

| Lubricant No.                                                  | 1     | 2     | 3      | 4      | 5     |
|----------------------------------------------------------------|-------|-------|--------|--------|-------|
| Composition, Percent by Wt.:                                   |       |       |        |        |       |
| Heavy residuum                                                 | 58.0  | 83.3  | 61.5   | 34.7   |       |
| Light distillate                                               | 40.0  | 14.7  | 36.5   | 31.5   |       |
| Oxidized residuum (cut-back)                                   | 0.0   | 0.0   | 0.0    | 33.3   |       |
| Paratac                                                        | 2.0   | 2.0   | 2.0    | 0.5    |       |
| Tests:                                                         |       |       |        |        |       |
| Viscosity, Saybolt Universal, seconds—                         |       |       |        |        |       |
| at 100° F.                                                     | 2,995 | 3,215 | 2,833  | 2,210  | 2,729 |
| at 210° F.                                                     | 145.5 | 153   | 148.1  | 147.5  | 123.5 |
| Viscosity Index                                                | 77.1  | 78.6  | 84.3   | 100.1  | 56.4  |
| Pour                                                           | —5    | 15    | —5     | 0      | 0     |
| Modified Penetration                                           | 355   | 353   | 354    | 350    | 348   |
| A. S. T. M. Bomb Oxidation Test, Pressure Drop, lbs. 100 hours |       |       | 19; 19 | 17; 18 |       |

As shown by the above table, Lubricant No. 4, which was prepared in accordance with this invention, had both a low pour point and a high viscosity index, whereas the straight mineral oil blends having pour points of the same order had much lower viscosity indices. In addition, the lubricant of this invention had excellent oxidation resistance, as shown by the A. S. T. M. Bomb Oxidation test, being equivalent in this respect to the commercial lubricant.

Table II shows the low temperature characteristics of the above lubricants as measured by the so-called GE Cold Starting Test. This test is used to determine the suitability of lubricants for use in the transmissions of washing machines. Since these machines are frequently stored in unheated places and used without warming up, the low temperature characteristics of lubricants employed for this purpose are very important, a great deal of trouble having been experienced with the electric motors burning out due to the excessive drag upon them during cold starting when lubricants of the prior art have been employed in the transmissions.

The equipment employed in the test is the transmission unit from a General Electric washing machine of the conventional agitator-wringer type, Washer Model AW-052, mounted on a test stand. In carrying out the test, the transmission is first thoroughly cleaned and charged with one and one-half pints of the test oil, and adjusted to consume 145 watts unloaded at room temperature with a 110 volt current supply. The test stand is then placed in a cold room maintained at about 29–33° F. for at least 16 hours, after which it is removed and a 90 volt current applied to the motor of the machine

25 with the agitator engaged. The power consumption is measured periodically under this set of conditions. Then the test is repeated in the same manner with a 160 watt adjustment at room temperature. The ability of the unit to start and the power consumption are indicative of the suitability of the lubricant for this purpose.

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835</p

2. A gear lubricant having substantially the following composition in per cent by volume:

|                                              |           |
|----------------------------------------------|-----------|
| Unoxidized mixed-base petroleum residuum,    |           |
| 720-740 SUS viscosity at 210° F.             | 33- 35    |
| Unoxidized naphthenic distillate, 55-65      | 5         |
| SUS viscosity at 100° F.                     | 31- 34    |
| Unoxidized naphthenic distillate, 75-125     |           |
| SUS viscosity at 100° F.                     | 15- 20    |
| Oxidized cylinder stock residuum,            |           |
| 55-75 penetration at 77° F.                  | 10 15- 20 |
| Foam inhibitor, 10% kerosine solution of     |           |
| dimethyl silicone polymer, parts per million | 50-150    |

3. A gear lubricant consisting essentially of a blend of at least about 25 per cent by weight of an unoxidized residual oil of low wax content having a viscosity of about 600-800 seconds Saybolt Universal at 210° F., at least about 35 per cent by weight of an unoxidized light distillate oil comprising in major proportion a naphthenic distillate oil having a viscosity of about 50-100 seconds Saybolt Universal of 100° F., and about 5-30 per cent by weight of an oxidized residuum having a penetration at 77° F. of about 30-100, obtained by blowing a paraffinic residual oil having a viscosity in the lubricating oil range.

4. A gear lubricant consisting essentially of a blend of about 25-40 per cent by weight of an unoxidized residual oil of low wax content having a viscosity of about 600-800 seconds Saybolt Universal at 210° F., about 35-65 per cent by weight of an unoxidized light distillate oil having a viscosity below about 200 seconds Saybolt Universal at 100° F. and comprising in major proportion a naphthenic distillate oil having a viscosity of about 50-100 seconds Saybolt Universal at 100° F., and about 5-30 per cent by weight of an oxidized residuum having 35 a penetration at 77° F. of about 40-90, obtained by

blowing a paraffinic residual oil having a viscosity in the lubricating oil range.

5. A gear lubricant consisting essentially of a blend of about 25-40 per cent by weight of an unoxidized residual oil of low wax content having a viscosity of about 700-800 seconds Saybolt Universal at 210° F., about 35-65 per cent by weight of an unoxidized light distillate oil having a viscosity below about 200 seconds Saybolt Universal at 100° F. and comprising in major proportion a naphthenic distillate oil having a viscosity of about 50-100 seconds Saybolt Universal at 100° F., and about 10-30 per cent by weight of an oxidized residuum having a penetration at 77° F. of about 55-75, obtained by blowing a paraffinic residual oil having a viscosity in the lubricating oil range.

6. A gear lubricant consisting essentially of a blend of about 25-40 per cent by weight of a predominantly paraffinic unoxidized residual oil of low wax content having a viscosity of about 600-800 seconds Saybolt Universal at 210° F., about 35-65 per cent by weight of an unoxidized light distillate oil having a viscosity below about 200 seconds Saybolt Universal at 100° F. and comprising in major proportion a naphthenic distillate oil having a viscosity of about 50-100 seconds Saybolt Universal at 100° F., and about 5-30 per cent by weight of an oxidized residuum having a penetration at 77° F. of about 55-75, obtained by blowing a paraffinic residual oil having a viscosity in the lubricating oil range.

#### References Cited in the file of this patent

##### UNITED STATES PATENTS

|           |              |               |
|-----------|--------------|---------------|
| 1,238,101 | Burch        | Aug. 28, 1917 |
| 1,831,614 | White et al. | Nov. 10, 1931 |
| 2,043,923 | Burwell      | Jan. 15, 1934 |
| 1,967,255 | Penniman     | July 24, 1934 |